

# UNITED STATES PATENT OFFICE.

FRANK A. FAHRENWALD, OF CLEVELAND, OHIO.

## ALLOY.

1,333,965.

Specification of Letters Patent. Patented Mar. 16, 1920.

No Drawing.

Application filed June 25, 1917. Serial No. 176,668.

*To all whom it may concern:*

Be it known that I, FRANK A. FAHRENWALD, a citizen of the United States, residing at Cleveland, in the county of Cuyahoga and State of Ohio, have invented a certain new and useful Improvement in Alloys, of which the following is a full, clear, and exact description.

This invention relates to alloys of beryllium, and has for its object the production of alloys of extreme lightness, combined with sufficient rigidity, tensile strength, and resistance to heat and oxidation for practical structural and mechanical purposes.

I have found that the alloys of beryllium possess properties more valuable in some ways than those of the similar and better known metals aluminum, magnesium, and calcium, and that certain of the valuable attributes of aluminum and magnesium (and to a smaller extent those of calcium) can be enhanced by the addition of beryllium thereto. Chief among the peculiar attributes of beryllium are its low specific gravity, its low atomic weight, its resistance to oxidation and chemical action, and its ability to form a close grained, impervious adherent oxid which forms an efficient protection against deterioration of any alloy in which it is contained. By combining this metal with other metals of low specific gravity but less immunity to oxidation it is possible to secure a substance of great lightness and permanence; while by the addition of small amounts of certain allied heavier metals it is possible to secure great rigidity, tensile strength, and mechanical permanence.

Alloys having these properties are of great importance in the construction of machines for aerial navigation and for the moving parts of high speed mechanism, such for example as the pistons of gasolene engines, as well as being of great desirability in connection with land and water vehicles and in most other places where metals are used. Pure beryllium alone is not well suited to these purposes on account of its softness and ductility, but if alloyed with certain other metals as herein pointed out its tensile strength and hardness are increased by an amount depending upon the nature and proportion of the other metal added; which nature and proportion are dependent upon the use contemplated and upon the value of that use which determines

to some extent the intrinsic value of the metals which can be employed therein.

For an alloy of extreme lightness I employ lithium and beryllium, the beryllium serving to protect the lithium from oxidation by moisture or heating and further action upon oxidation to produce upon the surface of the alloy a closely-adherent finely-textured, insoluble oxid which prevents further oxidation up to a lithium content of about 25% the corrosion tendency is apparently no greater than that of iron, while the specific gravity of such an alloy is only about 1.5.

If the proportion of lithium be increased to about 65% the alloy becomes as light as water and while becoming considerably more susceptible to oxidation in the presence of moisture, yet it can be protected by plating or covering sufficiently for many purposes. If the percentage of lithium be increased slightly above this point it becomes possible to add small quantities of aluminum or zinc to increase the hardness and strength while still retaining a specific gravity no greater than that of water.

Lithium alone is inapplicable to any mechanical or structural use owing to its softness and ductility and the fact that it decomposes water readily. It becomes valuable by reason of the great hardening effect and by reason of the shielding action of beryllium, both of which results are accomplished with less increase of specific gravity than would be possible with any other metal. The same is true of calcium, which, while normally of great softness and ductility and readily tarnished by moist air, becomes rigid and resistant upon alloying with beryllium. Besides the alloys of beryllium and calcium are extremely light in weight, and added stiffness can be imparted by the addition of a small percentage of copper or zinc or a larger percentage of aluminum. Thus the alloy of calcium 75% and beryllium 25% has a maximum hardness combined with a specific gravity of about 1.6, the hardness and stiffness being far greater than that of pure aluminum.

A more important use of beryllium is the hardening of aluminum or magnesium. Calcium has been proposed for alloying with aluminum for this purpose, but its effect is limited by the fact that aluminum will dissolve calcium only up to about eight per cent. by weight (according to L. Donski,

Zeitschrift für Anorganische Chemie, vol. 57 p. 185, 1908, Metallurgie, vol. 7, p. 572, 1911) which corresponds to only about six atomic per cent. and the resulting alloy is incapable 5 of being drawn into wire. Eight per cent. by weight of beryllium alloyed with ninety-two per cent. of aluminum corresponds to over twenty atomic per cent. of the whole with a correspondingly large effect upon the 10 properties of the resulting alloy. My investigations indicate a solubility of beryllium in aluminum even greater than this, with the production of malleable and ductile alloys.

15 Alloys of aluminum and beryllium have approximately the same specific gravity as the corresponding alloys of aluminum and calcium, but with enhanced strength, hardness, and stiffness and greater resistance to 20 corrosion. For example, the specific gravity of an alloy of Al 90, Be 10 is 2.5 and that of an alloy of Al 75, Be 25 is 2.4. Owing to the frequent occurrence together of aluminum and beryllium oxids I anticipate 25 a considerable degree of importance for this alloy.

Furthermore the addition of beryllium to the alloy of aluminum and calcium appears to increase the solubility of the calcium 30 therein, rendering the same more tough and malleable and less brittle and permitting the hardness to be increased still further.

For a lighter alloy of substantially the same strength I recommend beryllium and 35 magnesium, whose entire series is less than twice the specific gravity of water. These alloys also preferably possess a preponderating amount of magnesium, a composition of Mg 90, Be 10 being of apparently high commercial value. This alloy is also sufficiently 40 resistant to heat and moisture for most practical purposes, while further protection can be given by plating or coating.

The addition of beryllium also improves 45 the properties of calcium-magnesium alloys in the same way as alloys of aluminum and calcium. Outside of its beneficial effect as a solvent, the beryllium affords a peculiar advantage due to the large atomic effect 50 produced by a small weight per cent. coupled with an extremely low specific gravity.

Beryllium also makes excellent ternary 55 alloys with magnesium and copper or aluminum and copper, the copper being employed only in small quantities for increasing the hardness. Thus an alloy of aluminum 85, beryllium 10, and copper 5 will have a specific gravity of 2.8 and a hardness and tensile strength comparable with that 60 of bronze. Other metals such as titanium, vanadium, manganese, iron, cobalt, nickel or zinc can be used instead of or in connection with copper in this relation with the production of the same general results. Great

variations in solubility occur between these 65 metals, the limit of solubility of zinc being upward of thirty per cent. and that of titanium or vanadium very small. However only a small quantity of this hardening metal ought to be employed because of the 70 great comparative weight.

Another highly important use of beryllium is in connection with copper alone or high-copper alloys in the form of wires for 75 electrical heating or resistance elements, or in the form of heat treating boxes, furnace parts, burner nozzles, twyrs, and other articles subjected to high temperatures, since the superficial oxidation of the beryllium will protect the alloy from destructive 80 corrosion up to the melting point of the alloy and regardless of the time element. The same protective function also appears when beryllium is alloyed with other metals having an atomic weight between 48 and 66 although I consider the copper alloys superior 85 practically to those of the other members of that group. In general the alloys of beryllium with chromium, manganese, iron, cobalt and nickel, develop a considerable tendency 90 toward segregation as well as a coarsely crystalline structure which reduces their mechanical strength and prevents their being drawn into wire. Copper and zinc afford hardness to beryllium and its alloys 95 with less tendency toward these objectionable qualities, and the beryllium bronzes are more useful than the corresponding aluminum bronzes, being of higher melting point, more resistant to oxidation at high 100 temperatures, and of greater mechanical strength and hardness. These bronzes may contain aluminum, tin, manganese, nickel, etc., for hardening purposes without destroying the properties bestowed by beryllium. 105 However the proportion of beryllium ought to be either very small or very large, in order to produce a homogeneous alloy,—and the high cost of beryllium practically necessitates the use of the smaller proportion. In 110 fact the protective effect of beryllium upon copper, or other metals near copper in the same group, is strongly exhibited even though only two to five per cent. of the metal be present.

I have found that the metallic beryllium is a particularly efficient carrier of electric current and when produced in the form of drawn ductile wires is extremely useful in the construction of electrical apparatus 115 where large carrying capacity per unit of weight is required. The alloys containing over 90 per cent. of beryllium are more efficient in this respect than copper or aluminum. Wires of these beryllium alloys 120 can be used not only cold but are peculiarly applicable as resistance heating elements owing to their becoming 125

covered with an oxid coating at elevated temperatures. The alloys of beryllium-lithium, beryllium-calcium, beryllium-magnesium, beryllium-aluminum, beryllium-  
5 magnesium-calcium, beryllium-aluminum-calcium, and beryllium-lithium-aluminum (with or without the use of small proportions of heavier metals such as copper or zinc for hardening purposes) are of ex-  
10 treme value in aerial navigation, land and water transportation, and the rapidly moving parts of machinery, as will be obvious.

In preparing alloys of high beryllium content I have employed several methods. The  
15 pure element may be melted and the zinc, copper, aluminum, magnesium, lithium, calcium, etc., added directly to the molten bath, or a previously prepared alloy of beryllium and some other metal may be fortified  
20 or modified by further additions. Pure beryllium can be produced by the electrolysis of a fused salt in a manner similar to that for aluminum; and similarly by reducing a double salt or ore containing both beryllium and another metal an alloy may be produced directly. This method has been of  
25

greatest promise when using natural ores of beryllium, which usually contain aluminum.

Having thus described my invention, what I claim is:

1. An alloy composed of the metals aluminum and beryllium.
2. An alloy, comprising aluminum and one per cent. to ninety per cent. beryllium.
3. An alloy, comprising beryllium and 35 one or more metals in the class embracing aluminum.
4. An alloy possessing greater strength and less weight than aluminum, comprising aluminum and beryllium the aluminum 40 being in preponderating amount.
5. An alloy which is stronger, harder and of lighter weight than aluminum, consisting of aluminum and less than sixty-five per cent. beryllium.
6. An alloy, composed of one to twenty per cent. beryllium, with the balance chiefly aluminum.

In testimony whereof, I hereunto affix my signature.

FRANK A. FAHRENWALD.